

April 20, 1937.

O. F. GOTTLIEB

2,077,688

PISTON

Filed July 22, 1935

3 Sheets-Sheet 1



INVENTOR  
Oscar F. Gottlieb.

Charles Gottlieb Atty.

April 20, 1937.

O. F. GOTTLIEB

**2,077,688**

## PISTON

Filed July 22, 1935

3 Sheets-Sheet 2



Trenton  
Oscar J. Gottlieb.

by Charles St. Niles.

April 20, 1937.

O. F. GOTTLIEB

**2,077,688**

## PISTON

Filed July 22, 1935

3 Sheets-Sheet 3



Brenton  
Oscar F. Gottlieb.

by Charles W. Mills Atty.

## UNITED STATES PATENT OFFICE

2,077,688

## PISTON

Oscar F. Gottlieb, Lake Bluff, Ill., assignor to  
 Oakes Products Corporation, North Chicago,  
 Ill., a corporation of Michigan

Application July 22, 1935, Serial No. 32,533

2 Claims. (Cl. 309—14)

This invention relates to brazed pistons. More particularly the invention relates to pistons having a cast iron head brazed to a steel skirt to form a strong and rigid light weight piston.

5 It is an important object of this invention to provide pistons having a cast or forged head portion integrally united to a steel skirt.

Another important object of this invention is to provide pistons having a forged or cast head portion integrally brazed to a skirt portion formed from sheet metal.

10 A still further object of this invention is to provide a piston having a cast iron head portion with dependent ears formed thereon and brazed to a skirt formed from sheet steel.

Another important object of this invention is to provide brazed pistons from two different types of metal having similar coefficients of expansion.

15 A still further object of this invention is to provide a process of making pistons that includes the brazing of a skirt portion onto a head portion preferably in a reducing or hydrogen atmosphere.

20 Another object of this invention is to provide a method for manufacturing pistons that includes the steps of assembling a piston head portion and a piston skirt, placing a brazing wire at the junction between the piston and skirt and heating the assembly in a reducing atmosphere for melting the wire to integrally unite the head portion with the skirt portion.

25 30 Other and further objects of this invention will be apparent from the disclosures in the specification and the accompanying sheets of drawings which disclose preferred embodiments of this invention.

35 On the drawings:

Figure 1 is a vertical cross sectional view of a piston according to this invention.

Figure 2 is a plan view of a sheet metal disc 40 from which the piston skirt of this invention may be made.

Figure 3 is a cross sectional view of the disc shown in Figure 2 and indicating the manner in which the disc is stamped or drawn into a cup shaped member.

45 Figure 4 is a vertical cross sectional view of a cup shaped member formed from the disc shown in Figure 2 and illustrating the bottom of the cup shaped member that is cut away to form the piston skirt from the cup member.

50 Figure 5 is a plan view of a strip of sheet metal for forming a piston skirt according to an alternative method.

Figure 6 is an assembled view of the strip 55 shown in Figure 5.

Figure 7 is a vertical cross sectional view, with parts in elevation, showing the head portion of a piston according to this invention.

Figure 8 is a vertical cross sectional view, with parts in elevation, showing the manner in which the skirt portion and the head portion are assembled, and also showing the manner in which the brazing wire is positioned for the brazing operation.

Figure 9 is cross sectional view taken substantially along the line IX—IX of Figure 8.

Figure 10 is a fragmentary vertical cross sectional view of a brazed piston according to this invention, showing the braze between the head portion and the skirt portion.

Figure 11 is a side elevational view of a modified form of brazed piston according to this invention.

Figure 12 is a cross sectional view taken substantially along the line XIII—XII of Figure 11.

Figure 13 is a cross sectional view taken substantially along the line XIII—XIII of Figure 12.

As shown on the drawings:

In Figures 1 and 7 to 10 inclusive, the reference numeral 10 indicates a forged or cast iron piston head having two oppositely disposed lugs or ears 11 and 12 extending therefrom. Each ear 11 and 12 is provided with a horizontally disposed cylindrical boss portion 13 which may be drilled out to form openings 14 for receiving a wrist pin therethrough. The boss portions 13 are reinforced by webs such as 15 and 16 formed integrally on the inside of the lugs or ears 11 and 12 and extending from the boss portion 13 to the head 10.

35 As best shown in Figure 7, the head 10 has an annular flange 17 extending therefrom to define an annular shoulder 18 around the head 10.

As shown in Figure 1, a plurality of grooves 19 are formed in the periphery of the head 10 for receiving piston rings.

40 A steel skirt 20 is slipped over the ears 11 and 12 of the head 10 and around the flange 17 until it abuts the shoulder 18 of the head. The skirt 20 is formed according to the methods shown in Figures 2 to 6.

45 In Figure 2 the reference numeral 21 indicates a circular metal disc of sheet steel. As indicated in Figure 3, the metal disc 21 is spun or drawn into a cylindrical cup member 22. Any simple sheet metal stamping operation or spinning operation can be used to form a cylindrical cup from the disc 21.

50 As shown in Figure 4, the cup 22 is next formed into the piston skirt 20 by punching out a circular

55

metal disc 23 from the base of the cup to provide a circular opening 24. It is preferred to cut the metal disc 23 of smaller diameter than the diameter of the cup 22 so as to form an inturned flange 25 around the base of the piston skirt 20. The flange 25 adds rigidity to the piston skirt.

If desired, the piston skirt 20 may be formed according to the method illustrated in Figures 5 and 6. In Figure 5 the reference numeral 26 indicates a strip of sheet metal such as steel having a width of the desired height for the piston skirt 20 and a length sufficient to form the circumference of a piston skirt of the desired diameter. One end of the strip 26 has a dovetailed 15 groove 27 cut therein by any suitable stamping or cutting operation, while the other end of the strip 26 has a dovetailed tab 28 formed thereon for fitting into the groove 27.

The so-formed strip 26 is then bent around a 20 mandrel to form a cylinder 29 shown in Figure 6 with the dovetailed end 28 seated into the dovetailed groove 27 formed in the other end and with the edges of the strip in abutting relation. A brazing wire 30 is laid over the seam formed 25 between the interlocking ends of the cylinder 29 and the ends of the cylinder are then brazed together in the same operation involving the brazing of the head 10 to the piston skirt 20 as will be hereinafter described. While the wire 30 has 30 been shown to be placed on the outside of the cylinder 29, it should be understood that it can also be placed on the inside of the cylinder. It should also be understood that other forms of 35 interlocking tabs and grooves may be used in place of the tab 28 and the groove 27.

When the piston skirt 20 is slipped onto the head 10, the piston is then inverted as shown in Figure 8 and brazing wires 31 and 32, as shown in Figures 8 and 9, are placed over the flange 17 of 40 the head 10. The wires 31 and 32 are composed of copper, brass or bronze and are bent arcuately as shown in Figure 9, to fit around the flange 17 in abutting relation to the inside of the skirt 20. As shown in Figures 8 and 9, the wires 31 and 32 45 do not extend over the ears 11 and 12, but if desired the wires may be looped over these ears.

The piston is then inserted in the inverted position shown in Figure 8 in a brazing furnace where it is heated to a temperature above the melting 50 point of the wires 31 and 32. The copper or bronze forming the wires 31 and 32 is melted and flows by capillarity between the closely abutting surfaces of the piston skirt 20 and head 10. The molten metal even flows up around the ears 11 and 12 to form a braze between the ears and the side of the piston skirt.

The brazing is preferably carried out in a reducing atmosphere which may suitably be hydrogen or a mixture of gases relatively rich in hydrogen, carbon monoxide and nitrogen. Comparatively little oxygen should be present in the atmosphere of the brazing furnace if a satisfactory braze is to be obtained and the formation of scale 60 prevented.

If desired, the assembled parts of the piston 65 may be placed on a traveling conveyor with the piston head 10 contacting the conveyor. The assembled units are then run into a furnace having a reducing or hydrogen atmosphere and heated to a temperature sufficiently high to effect the brazing operation. Where copper brazing wires are used, the temperature should be about 2040° F. Where bronze wires are used, the temperature can be slightly lower, namely in the neighborhood of 1850° F. At these temperatures

and under a reducing condition, the brazing metal or alloy, upon melting, wets the surfaces with which it comes into contact, and flows by capillary action between the closely adjacent surfaces of the piston skirt 20 and the head 10 to form a 5 braze 33 (Figure 10) which extends around the entire periphery of the flange 17 and even up around the ears 11 and 12.

When the brazing operation is complete, the piston can be removed from the furnace through 10 a cooling chamber that is also supplied with a reducing or non-oxidizing atmosphere so that the metals of the piston may reach a sufficiently low temperature to prevent oxidation during the cooling 15 down period.

When the piston skirt 20 is formed according to the method disclosed in Figures 5 and 6, the brazing wire 30 of copper or bronze is disposed over the abutting edges of the strip 26 forming the cylinder 29 and melts down together with the 20 wires 31 and 32 to form an integrally united piston skirt during the same operation in which the piston skirt is united to the head.

When the brazed piston has cooled down, the boss portions 13 of the ears 11 and 12 may be 25 drilled as shown in Figure 1 to form openings 14, and at the same time circular openings 34 are also formed through the walls of the piston skirt 20, in alignment with the openings 14 of the bosses 13. When the wrist pins are thus inserted 30 through the openings 14 and 34 the surfaces of these openings form a bearing for the wrist pins.

In Figures 11, 12 and 13 there is illustrated a modified form of a piston according to this invention in which the reference numeral 40 indicates a forged or cast iron piston head having a pair of dependent ears 41 and 42 extending on opposite sides thereof. The ears 41 and 42 are provided with cylindrical boss portions 43 which may be drilled to provide openings 44 as shown 40 in Figure 12 for receiving a wrist pin.

Grooves 45 are formed around the periphery of the head 40 for receiving piston rings (not shown).

As shown in Figure 12, a web 46 is formed across 45 the inside of the head 40 and extends downwardly at both ends 46a thereof to reinforce the ears 41 and 42.

A depending flange 47 extends around the periphery of the head 40 at the lower end thereof 50 and has a somewhat smaller diameter than the diameter of the head 40 to form a shoulder 47a between the flange 46 and the head 40.

A piston skirt 48 is first formed according to either of the methods disclosed in Figures 2 to 6 55 and is then provided with a pair of spaced slots 49 and 50 on each side thereof to define two oppositely disposed strips 51 and 52 which are bent inwardly as best shown in Figure 13 to form reinforcing portions across the central portion 60 of the skirt 48. The excess metal is crimped to form beads 53 on each side of the reinforcing strips 51 and 52.

The central portions of the strips 51 and 52 are then cut away as shown at 54 for receiving the 65 ears 41 and 42 of the piston head. The piston skirt thus formed is slipped over the flange 46 of the piston head 40 until its end abuts the shoulder 47a thereon.

Brazing wires are then laid around the flange 70 47 with the piston assembly in an inverted position. Since the ears 41 and 42 extend through openings 54 formed in the strips 51 and 52 of the piston skirt, these ears are not united to the skirt and only one brazing wire need be looped 75

around the inside periphery of the flange 46 instead of using two individual wires as shown in Figures 8 and 9.

The piston with the brazing wire therein is 5 then brazed in a furnace in the same manner described in connection with Figures 1 and 8 to 10 to form a braze 55 around the periphery of the flange 47, thereby integrally uniting the piston skirt 48 with the head 40.

10 It should be understood that according to this invention pistons may be made from two different metals. I prefer however to use a cast head portion of grey iron and a skirt portion of mild steel. The brazing wires of copper, brass or bronze have 15 great affinity for the cast iron head and, when placed in the piston as described above, readily flow by capillary action between all contacting portions of the iron head and the steel skirt to integrally unite the skirt to the head. The resulting piston is much stronger than a cast iron 20 piston and can be made of light gauge metal thereby producing a product of about the same weight as aluminum pistons. At the same time, however, the pistons of this invention have a 25 coefficient of expansion about the same as the coefficient of expansion of the engine block and thus need not be loosely fitted into the block as is the case when aluminum pistons are used.

It has been found by tests that the steel skirts 30 cannot be torn away from the head portion without heating the piston above the melting point of the brazing material. Since the temperatures of an internal combustion engine never reach 35 temperatures at which the brazing material becomes molten, there is no danger of the brazed pistons of this invention ever separating during use.

I am aware that many changes may be made

and numerous details of construction may be varied through a wide range without departing from the principles of this invention, and I, therefore, do not purpose limiting the patent granted hereon otherwise than necessitated by the prior 5 art.

I claim as follows:

1. A composite piston comprising a cast iron head portion having depending ears extending therefrom on opposite sides thereof, said ears 10 carrying apertured bosses on the ends thereof for receiving the ends of a wrist pin, a cylindrical steel skirt portion telescoped on part of the head portion and having a pair of spaced cuts therein on each side thereof defining web portions there- 15 between, said web portions being indented to reinforce the skirt and having parts thereof cut away to receive the depending ears of the head and a thin film of a copper containing brazing material between and alloyed with the telescoped 20 portions of the head and skirt to integrally unite said portions.

2. A composite internal combustion engine piston comprising a cast iron head portion including a reduced section, a steel skirt fitted about 25 and telescoped by said reduced section and having its outer surface flush with that of the head portion, a thin film of a brazing material between and alloyed with the telescoped portions of the head and skirt to integrally unite said portions, 30 said head portion having depending ears extending therefrom on opposite sides thereof forming wrist pin bosses, said skirt portion having a pair of spaced cuts therein on each side thereof defining web portions therebetween and said web 35 portions being indented to reinforce the skirt.

OSCAR F. GOTTLIEB.